

## UNITED STATES PATENT OFFICE

2,088,628

## MANUFACTURE AND USE OF TEXTILE THREADS

William Whitehead, Cumberland, Md., assignor to Celanese Corporation of America, a corporation of Delaware

No Drawing. Application February 3, 1936,  
Serial No. 62,166

27 Claims. (Cl. 117—21)

This invention relates to the manufacture of crepe threads from filaments of cellulose acetate or other organic derivatives of cellulose and to the production of fabrics therefrom.

5 This application is a continuation-in-part of my applications Ser. No. 703,427 filed Dec. 21, 1933 and S. No. 746,135 filed September 29, 1934.

Fabrics exhibiting crepe effects have long been obtained by employing in their construction highly twisted yarns of natural silk in the gummed state, the crepe effects appearing mainly when fabrics so formed are subjected to an aqueous scouring treatment. The fabrics obtained by this process are highly valued on account of their 10 pleasing appearance and handle. The production of crepe fabrics in an analogous manner by the use of crepe threads of cellulose acetate has, however, been accompanied by difficulties. Generally, the crepe effect obtained by simply applying 15 to a cellulose acetate thread a twist of the order of that commonly employed in connection with natural silk, weaving the twisted threads into a fabric and scouring the latter, is very unsubstantial and not comparable with that obtained with natural silk or regenerated cellulose 20 artificial silk.

In accordance with the present invention highly twisted crepe threads of organic derivative of cellulose filaments are produced from threads of 25 filaments of organic derivative of cellulose by crepe twisting in a single stage and during the insertion of the crepe twist steaming the threads, moisture preferably being present; i. e. the steam is applied to the travelling thread over at least 30 a portion of that part of its track in which twisting is actually taking place. Good results may be obtained by steaming at above 95° C. Steam temperatures in the neighborhood of 100° C., are especially to be recommended. The steam preferably contains a substantial amount of moisture 35 although good results may be obtained with dry steam.

This invention is of especial value and will be more particularly described in connection with 40 the production of crepe threads of filaments of cellulose acetate.

In this way it has been found possible to produce crepe threads which yield fabrics exhibiting remarkably good crepe effects. Moreover, 45 by this new process cellulose acetate crepe threads may be produced which have an average strength very much greater than that of cellulose acetate crepe threads produced by a simple twisting operation without the steam treatment 50 during twisting. Further, apart from the great

advantage of a stronger resultant thread, the twisting operation itself is greatly facilitated in that twisting may satisfactorily be accomplished under conditions of twist and spindle speed which in the absence of the steaming would give rise 5 to frequent thread breakage and render impossible the insertion of the desired twist or at least result in a very weak and useless thread.

The initial thread may already be twisted to a small degree, for example up to 10 turns per 10 inch, e. g. 2-5 turns per inch, or to such other small degree as is commonly applied in the production of cellulose acetate threads by dry spinning cellulose acetate solutions and winding and twisting the resultant filaments on a cap-twisting 15 device or other twisting and/or winding device.

The threads may consist of substantially continuous filaments of cellulose acetate or they may contain discontinuous filaments of cellulose acetate, the length of which may vary within wide limits. For example the threads may be those spun from a mass of discontinuous filaments or those prepared in the manner described in British patent specifications Nos. 424,683, 424,752, 25 424,830 and 424,879.

If desired, the filaments of the threads may contain water-insoluble compounds, whether 30 compounds of pigment-like character in such form as materially to modify the lustre of the filaments (e. g. barium sulphate or titanium dioxide), or loading metal compounds, for example tin compounds.

In carrying out the new process, twisting may be effected on a device of the kind in which the 35 thread is drawn off over the end of a rotating package through a guide fixed substantially in line with the axis of rotation of the package and is thereafter wound on a bobbin or the like, the thread being passed on its way from the guide to the bobbin, through steam under conditions such that moisture is present. In this way the thread is subjected to the action of the steam and moisture during the actual application of twist.

The twisting spindle, the guide fixed in line 40 with the axis of the spindle, and the steaming device should be so arranged that the twist resulting from the rotation of the package is at least partly inserted while the thread is under the influence of steam. For example, when twisting as the thread is drawn off over the end of a rotating package, if the freedom of the 45 thread to rotate within the balloon guide or other guide preceding or forming part of the steaming 50 55

device, is unduly restricted, e. g. by causing the thread to change direction materially at the guides, the insertion of twist while the thread is under the influence of the steam may be restricted to an undesirable extent, or substantially prevented, and the resulting crepe threads may not have the valuable properties which may otherwise be secured. Thus, when using a twisting device of the kind in which thread is drawn off over the end of a rotating package, it is advantageous to arrange that the path of the thread after leaving the balloon guide and through the steaming device, is substantially in line with the axis of the twisting spindle.

15 On the other hand, any other suitable crepe twisting device may be employed. For example, a ring twister may be used for the crepe twisting of thread consisting of discontinuous cellulose acetate filaments. In the case of a ring twister, where twisting is effected as the thread is wound on to a rotating package, the thread passing through steam on its way from the let-off device to the twisting spindle, a change of direction at the point where the thread leaves the steaming device is of less importance as the thread remains under the influence of the steam for a short time after leaving the steaming device.

If desired, the above-mentioned twisting devices, in which the thread is drawn off over the end of a rotating package, may be provided with a device which restricts the ballooning of the thread or the tendency of twist to run back to the package. As examples of such devices may be mentioned flyers and the floating ring device described in British Patent No. 304,806 of British Celanese Limited and others. The latter device is of particular value when the thread to be twisted is of very low twist, for example of less than about 1 turn per inch.

40 Steaming may conveniently be effected by allowing the thread to pass through a suitable chamber supplied with steam under such conditions that moisture is present.

Thus, a vertical twisting spindle of the type in which thread is drawn off upwardly over the end of a rotating package through a guide substantially in line with the axis of the spindle, may be provided with a small chamber situated vertically above the spindle. The chamber is provided with 45 small holes, top and bottom, to permit passage of the thread, and also with a steam inlet. If desired, a single steam chamber may be arranged to serve a number of spindles, being provided with inlet and outlet holes for the thread of each spindle. Such an apparatus may conveniently consist of a horizontal pipe mounted over a row of spindles and provided with eyes of porcelain, stainless steel, or other suitable material at appropriate points on top and bottom for the entrance and exit of the threads. The diameter of the pipe is sufficient to afford the thread the requisite length of travel in the steam. Steam may be admitted to the pipe at one point or at 50 more than one point as may be necessary according to the length of the pipe, to secure sufficiently uniform conditions of steaming as between the threads from the different spindles.

At the point at which the thread from the twisting spindle enters the steaming device, it is advantageous to arrange a free escape of steam on to the thread as it is drawn off from the spindle. A shield, for example in the form of a funnel, may, if desired, be fitted around the thread approaching the steaming device in order to

75 maintain an atmosphere of steam around the thread.

The presence of the desired moisture may be assured by arranging for condensation of steam in the steaming device. Dry steam may be passed through water so as to saturate the steam and the requisite moisture produced by cooling in the steaming device.

Another method of ensuring the presence of moisture is to wet the thread with water; for example the bobbins of thread may be wetted before the twisting operation or better, water may be applied to the thread, by means of a wick or other device, after the thread leaves the spindle and prior to its entering the steaming device. The water may contain a substance which facilitates wetting of the thread by water.

Steam at about atmospheric pressure, e. g., slightly above atmospheric pressure, is conveniently employed. If desired, however, the steaming may be effected with steam at any desired super-atmospheric pressures, e. g., steam at 10-25 lbs. per square inch.

A steaming treatment of relatively short duration such as may be secured by passing the yarn at a speed of from 2 to 10 metres per minute through 3" of steam has been found to give satisfactory results. Lengthier treatments may, however, be employed, for example the yarn may be passed at the said speeds through 6 to 12" or more of steam.

The cellulose acetate filaments of the threads very readily undergo stretching when the threads are twisted under the influence of the steam and moisture. The amount of stretch may be measured by comparing the original thread denier with the final thread denier (after untwisting). It has been found that when a cellulose acetate thread is crepe twisted by the process involving steaming during twisting in one operation so as to produce a crepe thread of good strength and creping properties, the denier of the resultant thread is, in general, owing to imparted stretch, less and even substantially less than if the thread is simply crepe twisted without the steam treatment. The stretch imparted to the filaments of the threads during the twisting operation may for example be of the order of 5-25% of their original length, and particularly 10-20%. The degree of stretching of the filaments of the thread may be such that the final denier of the crepe twisted thread is not much in excess of or is even the same or less than the denier of the thread prior to twisting. For example the stretch may be such that the denier of the crepe twisted thread is from 95 to 115%, particularly 100 to 110% of that of the thread before crepe twisting, especially in the case of threads having an original denier of 150 or less. Good crepe fabrics may however be obtained when the final denier is still greater, for example up to 120% of that of the thread before twisting when threads having a denier about 200 are employed.

The degree of twist applied in accordance with the new process may vary within wide limits. A feature of the process is that it enables a high degree of twist to be applied without such a great weakening of the thread as is almost invariably experienced when cellulose acetate crepe threads are prepared without steaming. The process, moreover, permits the insertion of twists which are impossible of attainment without the steaming owing to breakage of the thread. This is important since it enables crepe fabrics to be produced having very pronounced crepe effects.

The crepe figure can be regulated according to requirements. The degree of twist desirable in any particular case depends upon the denier of the thread. For example with threads of 165 5 denier twist of about 70 to 75 turns per inch is desirable, and with threads of 115 denier twist of about 85 to 90 turns per inch. With these indications it is a simple matter to determine the desirable twists for threads of other deniers. 10 The denier numbers given are those of the threads after crepe twisting.

As indicated above, the new process enables highly twisted cellulose acetate threads of high creping power to be produced. In these new 15 threads the filaments are extremely closely packed, a feature to which their good creping power may be attributed. For example, the filaments may be so closely packed that the apparent specific gravity of the thread as determined 20 from the diameter and denier is more than 85%, e. g. 85 to 90% of the actual specific gravity of the filaments, and that distortion of the cross-section of at least some of the filaments has occurred during the process of twisting. The 25 filaments of the thread, however, are not stuck together and can be separated upon untwisting. Moreover, the new cellulose acetate crepe threads are smooth and cylindrical as opposed to the rough feel and helical form of a cellulose acetate 30 thread or a viscose thread which has been crepe twisted in the ordinary way. Further, in comparison with these latter threads, the smooth cylindrical cellulose acetate crepe threads exhibit much less tendency to snarl or kink. These 35 characteristics distinguish the new cellulose acetate crepe threads.

While the new process enables production of threads which yield satisfactory crepe effects without a special treatment, other than the twisting and steaming treatment characteristic of the 40 process, other devices and treatment may, if desired, be employed further to improve the properties of the crepe threads and/or fabrics produced therefrom. For example, the crepe threads 45 may be sized at any suitable stage of their manufacture, for example in the course of winding on to the bobbin from which twisting is effected. In the connection, particular mention may be made of sizing materials selected in accordance with 50 the considerations laid down in British patent specification No. 348,589. For example a casein, egg-albumen, or other size which is not very readily removed by aqueous treatments may be employed. Another size which may be employed 55 is a drying oil, if desired one which has been partially oxidized, e. g. boiled or blown linseed oil.

The highly twisted crepe threads may be incorporated in the fabrics in various ways, for 60 example the weft alone may be wholly or partially composed of such threads or the warp may also contain them. Valuable fabrics may be produced by employing warp threads of relatively low twist and in the weft both crepe threads having a 65 left-hand twist and crepe threads having a right-hand twist, pairs of threads of left-hand twist alternating with pairs of threads of right-hand twist.

If desired the cellulose acetate crepe threads 70 may be associated in the fabrics with highly twisted crepe threads of other materials, e. g. of natural silk or regenerated cellulose or produced by other processes. Where the fabrics contain threads of low twist these may wholly be of 75 cellulose acetate or wholly or in part of other

materials, e. g. natural silk or regenerated cellulose.

Fabrics containing highly twisted crepe threads prepared in accordance with the invention may subsequently be given a hot aqueous treatment, 5 for example in the manner commonly adopted in connection with fabrics comprising highly twisted yarns of natural silk. Enhanced crepe effects may be obtained by means of hot aqueous treatments at or near the boiling point. 10

An important characteristic of fabrics exhibiting crepe effects produced in accordance with this invention is that unlike crepe fabrics heretofore produced, they do not shrink substantially when washed or otherwise treated with aqueous liquids, 15 nor do they tend to develop spots when subjected locally (such as by rain) to aqueous liquids. Therefore garments or other articles made of such fabric may be laundered in the ordinary way without recourse to dry cleaning. 20

While this invention has been described in particular connection with cellulose acetate, it is applicable for use with yarns or threads made of other organic derivative of cellulose, such as cellulose formate, cellulose propionate, cellulose 25 butyrate, cellulose acetate-propionate or other organic esters of cellulose, or cellulose ethers such as ethyl cellulose or benzyl cellulose.

It is to be understood that the foregoing detailed description is merely given by way of 30 illustration and many alterations may be made therein without departing from the spirit of my invention.

Having now particularly described and ascertained in the nature of my said invention and in 35 what manner the same is to be performed, I declare that what I claim is:—

1. Process for the production of highly twisted crepe threads of filaments of an organic derivative of cellulose, which comprises steaming threads 40 of filaments of an organic derivative of cellulose and crepe twisting the threads in a single stage while the threads are subjected to the action of the steam.

2. Process for the production of highly twisted 45 crepe threads of filaments of an organic derivative of cellulose, which comprises steaming threads of filaments of an organic derivative of cellulose under conditions such that moisture is present and crepe twisting the threads in a single stage 50 while the threads are subjected to the action of the steam.

3. Process for the production of highly twisted crepe threads of filaments of an organic derivative 55 of cellulose, which comprises passing threads of filaments of an organic derivative of cellulose through a chamber maintained full of steam under conditions such that moisture is present, and crepe twisting the threads in a single stage while the threads are being steamed.

4. Process for the production of highly twisted crepe threads of filaments of an organic derivative of cellulose, which comprises crepe twisting threads of filaments of an organic derivative of cellulose in a single stage and during the insertion of the crepe twist steaming the threads 65 under conditions such that moisture is present.

5. Process for the production of highly twisted crepe threads of filaments of an organic derivative of cellulose which comprises steaming 70 threads of filaments of an organic derivative of cellulose with steam at above 95° C. under conditions such that moisture is present, and crepe twisting the threads in a single stage while the threads are being steamed. 75

6. Process for the production of highly twisted crepe threads of cellulose acetate filaments, which comprises steaming threads of cellulose acetate filaments and crepe twisting the threads in a single stage while the threads are subjected to the action of the steam. 5
7. Process for the production of highly twisted crepe threads of cellulose acetate filaments, which comprises steaming threads of cellulose acetate filaments under conditions such that moisture is present and crepe twisting the threads in a single stage while the threads are being steamed. 10
8. Process for the production of highly twisted crepe threads of cellulose acetate filaments, which comprises passing threads of cellulose acetate filaments through a chamber maintained full of steam under conditions such that moisture is present, and crepe twisting the threads in a single stage while the threads are being steamed. 15
9. Process for the production of highly twisted crepe threads of cellulose acetate filaments, which comprises crepe twisting threads of cellulose acetate filaments in a single stage and during the insertion of the crepe twist steaming the threads under conditions such that moisture is present. 20
10. Process for the production of highly twisted crepe threads of cellulose acetate filaments, which comprises steaming threads of cellulose acetate filaments with steam at above 95° C. under conditions such that moisture is present, and crepe twisting the threads in a single stage while the threads are being steamed. 25
11. Process for the production of highly twisted crepe threads of cellulose acetate filaments, which comprises steaming threads of cellulose acetate filaments with steam at substantially 100° C. under conditions such that moisture is present, and crepe twisting the threads in a single stage while the threads are being steamed. 30
12. Process for the production of highly twisted crepe threads of cellulose acetate filaments, which comprises steaming threads of cellulose acetate filaments under conditions such that moisture is present and crepe twisting the threads in a single stage while the threads are being steamed, the filaments of the threads being stretched from 5 to 25% of their original length while the twist is being inserted. 35
13. Process for the production of highly twisted crepe threads of cellulose acetate filaments, which comprises steaming threads of cellulose acetate filaments under conditions such that moisture is present and crepe twisting the threads in a single stage while the threads are being steamed, the filaments of the threads being stretched while the twist is being inserted so that the denier of the crepe twisted threads is 95% to 125% of that of the threads before crepe twisting. 40
14. Process for the production of highly twisted crepe threads of cellulose acetate filaments, which comprises crepe twisting threads of cellulose acetate filaments in a single stage by drawing them off over the end of a rotating package, and steaming the threads by passing them through a chamber maintained full of steam under conditions such that moisture is present, so that twisting is inserted while the threads are passing through the steam chamber. 45
15. Process for the production of highly twisted crepe threads of cellulose acetate filaments, which comprises crepe twisting threads of cellulose acetate filaments in a single stage as they are wound

on to a rotating package and steaming the threads by passing them through a chamber maintained full of steam under conditions such that moisture is present, so that twist is inserted while the thread is being steamed. 5

16. Process for the production of highly twisted crepe threads of cellulose acetate filaments, which comprises crepe twisting threads of cellulose acetate filaments in a single stage by drawing them off over the end of a rotating package, and steaming the threads by passing them through a chamber maintained full of steam at substantially 100° C. under conditions such that moisture is present, so that twist is inserted while the threads are passing through the steam chamber. 10

17. Process for the production of highly twisted crepe threads of cellulose acetate filaments, which comprises crepe twisting threads of cellulose acetate filaments in a single stage as they are wound on to a rotating package, and steaming the threads by passing them through a chamber maintained full of steam at substantially 100° C. under conditions such that moisture is present, so that twist is inserted while the thread is being steamed. 15

18. Process for the production of highly twisted crepe threads of cellulose acetate filaments, which comprises steaming threads of cellulose acetate filaments under conditions such that moisture is present and crepe twisting the threads in a single stage while the threads are being steamed, there being applied a minimum crepe twist determined according to the denier of the crepe threads after twisting, said minimum being 70 turns per inch for crepe threads of 165 denier or 85 turns per inch for crepe threads of 115 denier. 20

19. Highly twisted crepe threads of filaments of an organic derivative of cellulose, said filaments being so closely packed that the threads have an apparent specific gravity of above 85% of the actual specific gravity of the filaments. 25

20. Highly twisted crepe threads of cellulose acetate filaments, said filaments being so closely packed that the threads have an apparent specific gravity of above 85% of the actual specific gravity of the filaments. 30

21. Highly twisted crepe threads of cellulose acetate filaments, said filaments being so closely packed that the threads have an apparent specific gravity of 85% to 90% of the actual specific gravity of the filaments. 35

22. A smooth, cylindrical, highly twisted crepe thread of filaments of an organic derivative of cellulose, in which the filaments are so closely packed that the apparent specific gravity of the thread is more than 85% of the actual specific gravity of the filaments. 40

23. A smooth, cylindrical, highly twisted crepe thread of cellulose acetate filaments, in which the filaments are so closely packed that the apparent specific gravity of the thread is more than 85% of the actual specific gravity of the filaments. 45

24. A smooth, cylindrical, highly twisted crepe thread of cellulose acetate filaments, in which the filaments are so closely packed that the apparent specific gravity of the thread is 85 to 90% of the actual specific gravity of the filaments. 50

25. A smooth, cylindrical, highly twisted crepe thread of cellulose acetate filaments, in which the filaments are so closely packed that the apparent specific gravity of the thread is more than 85% of the actual specific gravity of the filaments, said thread having a minimum twist therein de. 55

terminated according to the denier of the crepe twisted thread, said minimum being 70 turns per inch for a crepe thread of 165 denier or 85 turns per inch for a crepe thread of 115 denier.

26. A highly twisted crepe thread of filaments of an organic derivative of cellulose, said fila-

ments being so closely packed that the thread is smooth and cylindrical.

27. A highly twisted crepe thread of cellulose acetate filaments, said filaments being so closely packed that the thread is smooth and cylindrical. 5

WILLIAM WHITEHEAD.